

## UNITED STATES PATENT OFFICE

2,148,404

## PRODUCTION OF ALKALI METALS

Harvey N. Gilbert, Niagara Falls, N. Y., assignor  
to E. I. du Pont de Nemours & Company, Wil-  
mington, Del., a corporation of Delaware

No Drawing. Application March 11, 1936,  
Serial No. 68,275

4 Claims. (Cl. 204—21)

This invention relates to the electrolysis of alkali metal compounds to produce alkali metals and other valuable products and more particularly to electrolysis processes which utilize liquid metal electrodes.

Various methods for electrolysis of alkali metal compounds either in the fused state or in aqueous solutions with the use of circulating liquid metal electrodes are well known. An example of this is the well-known Castner cell used for the production of caustic soda, wherein mercury serves as the cathode for the electrolysis of aqueous sodium chloride solution. In processes of this nature the alkali metal released at the liquid metal cathode alloys therewith and the liquid alloy then is circulated either to react chemically with water or other substances to produce caustic soda or other sodium compounds.

A number of methods have been proposed for producing metallic sodium or sodium compounds by the use of a two-cell system employing a liquid metal electrode whereby a fused sodium salt is first electrolyzed with a liquid metal cathode to form the sodium alloy and this liquid sodium alloy then is used as anode in a cell employing a fused sodium compound as electrolyte, e. g., caustic soda, whereby metallic sodium is released at the cathode. This method of producing sodium has not enjoyed any substantial commercial use and so far as I am aware is not commercially used at the present time. A significant disadvantage of this two-cell system of producing sodium has been the excessively high temperatures. These high temperatures, e. g., 350° C. or higher make it impractical to employ mercury as liquid electrode because of the high vapor pressure of mercury at such elevated temperatures. Further disadvantages of the high temperatures are that the working life of the equipment is seriously shortened because of the tendency of rapid corrosion at high temperatures, relatively massive and expensive equipment is required, and there is considerable loss of energy in the form of radiated heat.

Considerable advantage would be secured in the production of alkali metal, e. g., metallic sodium, if an alkali metal liquid alloy were first produced from electrolysis of an aqueous electrolyte and this alloy were then utilized as anode in a non-aqueous secondary cell which may be operated at a low temperature. In such arrangement, mercury (or alkali metal amalgam) would be a suitable metal to serve as the liquid electrode. So far as I am aware, no one heretofore has prepared a commercially feasible method of

doing this. It has been proposed to electrolyze aqueous salt solution with a mercury cathode and employ a second cell having a liquid ammonia solution of salt as electrolyte, where the amalgam resulting from the first electrolysis serves as anode. However, this method has not proved practicable for commercial operation, partly because of the difficulties attending the use of liquid ammonia solution as electrolyte.

An object of the present invention is to provide a practicable method whereby an aqueous solution of an alkali metal compound may be electrolyzed with a liquid metal cathode to produce a liquid alkali metal alloy and that alloy be utilized as anode in an electrolytic operation to produce alkali metal, e. g., metallic sodium. A further object is to provide a commercially feasible method for producing sodium metal or other alkali metal by electrolysis utilizing an alkali metal amalgam as anode at temperatures at which the vapor pressure of mercury is relatively low. Other objects will be hereinafter apparent.

The above objects are accomplished in accordance with the present invention by producing alkali metal amalgam by electrolysis of an aqueous alkali metal compound solution with a mercury (or amalgam) cathode and using the amalgam so produced as anode in electrolysis of a substantially anhydrous fused mixture of alkali metal hydroxide and alkali metal halide. I have discovered that exceptionally low-melting mixtures of alkali metal hydroxides and halides may be prepared which permit electrolysis in the fused state at temperatures at which the vapor pressure of mercury is relatively low. For example an eutectic mixture consisting of about 55% of sodium hydroxide and about 45% of sodium iodide (which is my preferred electrolyte for the production of sodium) has a melting point of about 225° C. and this mixture may be fused and utilized as molten electrolyte at temperatures of for example 230–250° C. At such relatively low temperatures, the vapor pressure of mercury is less than 1/10 atmosphere.

In one method of practicing the present invention for the production of sodium which is given by way of example, an aqueous solution of sodium chloride is electrolyzed in a cell having a flowing stream of mercury or sodium amalgam as cathode. As a result of this electrolysis, chlorine is liberated at the anode and means are provided for removing the gaseous chlorine as formed. Sodium liberated at the cathode unites with the mercury to form amalgam, so that the liquid

cathode flowing from the cell is richer in sodium than the mercury or amalgam entering the cell. The concentration of sodium in the amalgam leaving the cold cell may vary widely; a concentration of around 0.1 to 0.2% by weight is suitable. The liquid amalgam leaving the cell is led to a second cell in which the amalgam is utilized as anode. Preferably, the amalgam flows constantly through the second cell. The second cell employs as electrolyte the fused, eutectic mixture of sodium hydroxide and sodium iodide which contains about 55% by weight of sodium hydroxide and 45% by weight of sodium iodide and has a melting point of about 225° C. The temperature of this fused electrolyte is maintained at about 240-250° C. The cathode in this second cell may be made of iron or steel or other suitable conductive material. The electrolysis in the second cell results in constant removal of sodium from the flowing amalgam anode and the liberation of molten sodium metal at the cathode. The molten sodium, having a lower specific gravity than that of the electrolyte, rises towards the surface and suitable collecting means are provided above the cathode for entrapping the rising sodium and conducting it out to a closed receiver so that it is kept out of contact from the air. From time to time the collected sodium may be removed from the receiver. In addition to the above described eutectic mixture of sodium hydroxide and sodium iodide, other mixtures of these two compounds and various other mixtures of alkali metal hydroxides and alkali metal halides may be used as electrolytes according to my invention for the recovery of alkali metal from a liquid alkali metal alloy which serves as anode. If it is desired by means of such electrolysis to liberate a single alkali metal at the cathode, a fused electrolyte containing the hydroxide and a halide of that metal is employed. If it is desired to release a mixture of two or more alkali metals at the cathode, I would employ a fused electrolyte containing the corresponding hydroxides and halides preferably having the proportions of the alkali metals in the electrolyte at least roughly equivalent to the proportions in which these metals occur in the alkali metal amalgam anode. The selection of the halide to be mixed with the hydroxide and the proportions thereof will be determined chiefly by the temperature at which it is desired to operate the electrolytic cell. When using a mercury base anode, I prefer to employ an electrolyte which has a melting point not greater than about 300° C. With such an electrolyte the cell may be operated at temperatures slightly above 300° C., e. g. up to 310° C., at which temperatures the vapor pressure of mercury is around one-third of an atmosphere and hence the loss in mercury due to vaporization at ordinary pressures is small. If the melting point of the electrolyte is not over 250° C. the cell may be operated at temperatures sufficiently low that the vapor pressure of the mercury is not over about one tenth of an atmosphere, under which conditions there is little or no loss of mercury due to vaporization. Obviously various fused mixtures containing an alkali metal hydroxide and one or more alkali halides may be made up to obtain mixtures having various melting points over a wide range. To obtain mixtures having minimum melting points, I prefer to use substantially eutectic mixtures of these substances. In addition to the eutectic mixture of sodium hydroxide and sodium iodide which

has been mentioned above, the eutectic mixtures shown in the following table illustrate the variety of compositions which may be utilized to produce electrolytes having relatively low melting points:

| Eutectic mixture:         | Melting point (° C.) | 5  |
|---------------------------|----------------------|----|
| NaOH (79 molar %) + NaBr  | 260                  |    |
| KOH (72 molar %) + KI     | 250                  |    |
| KOH (65 molar %) + KBr    | 300                  |    |
| LiOH (45.5 molar %) + LiI | 180                  |    |
| LiOH (45 molar %) + LiBr  | 275                  | 10 |
| LiOH (63 molar %) + LiCl  | 290                  |    |

In its broader aspects, my invention relates to the electrolysis of a low-melting mixture of alkali metal hydroxide and alkali metal halide, utilizing a liquid alkali metal alloy as anode, so as to liberate alkali metal at the cathode. In order to obtain a sufficiently low melting point, the mixture of alkali metal hydroxide and halide may be an eutectic mixture or some mixture approximating or approaching the eutectic, i. e., a mixture having a melting point lower than that of its lowest melting component. The invention is not restricted to using alkali metal amalgam as the anode, since other low melting alloys of alkali metals are utilized for this purpose. Examples of such are "Woods metal" and other similar alloys of bismuth, lead, tin and/or cadmium. It is preferable, however, in most cases to use an amalgam electrode.

In carrying out the herein described process in a continuous manner over extended periods of time to produce alkali metals I have found that substantially no decomposition of the fused electrolyte occurs. The composition of the electrolyte remains substantially unchanged over extended periods of time and there is no evidence of anodic oxidation of the halide. For example, in a bath containing iodide, there is no formation of either iodate or per iodine. Hence the cell may be operated practically indefinitely without changing or replacing the electrolyte or readjusting the composition thereof.

In practicing the present invention, I prefer to utilize the method and apparatus disclosed and claimed in my copending application filed of even date herewith, whereby the liquid metal electrode is applied on the cell in the form of a thin film on a moving metal surface. In the preferred form of this method as disclosed in the aforesaid copending application the liquid alkali metal amalgam anode is flowed through a reservoir in the lower portion of the cell while the fused electrolyte floats on the surface of the amalgam in the reservoir. A disc rotating on its horizontal axis or other suitable moving surface is arranged partly immersed in the reservoir of amalgam and partly projecting into the electrolyte. By this means the disc is coated with a film of the amalgam and the rotation of the disc constantly brings a thin film of the amalgam from the reservoir into contact with the electrolyte, returning a thin film of amalgam from which a portion of the alkali metal has been removed by electrolytic action.

I claim:

1. A process for the recovery of an alkali metal from an alloy of said metal having a melting point not higher than about 100° C. comprising employing said alloy in the liquid state as anode in an electrolytic cell which contains as electrolyte a fused mixture of alkali metal hydroxide and alkali metal halide having a melting point below 300° C.

2. A process for the recovery of an alkali metal from an alkali metal amalgam comprising employing said amalgam as anode in an electrolytic cell which contains as electrolyte a fused mixture of alkali metal hydroxide and alkali metal halide, said mixture having a melting point below 300° C.

3. A process for the recovery of an alkali metal from an alkali metal amalgam comprising employing said amalgam as anode in an electrolytic

cell which contains as electrolyte a fused, substantially eutectic mixture of an alkali metal hydroxide and an alkali metal halide.

4. A process for the recovery of sodium from sodium amalgam comprising employing said amalgam as anode in an electrolytic cell which contains as electrolyte a fused eutectic mixture of sodium hydroxide and sodium iodide.

HARVEY N. GILBERT.